

# UNITED STATES PATENT OFFICE.

ANDREW THOMA, OF CAMBRIDGE, MASSACHUSETTS, ASSIGNOR TO NORTH AMERICAN CHEMICAL COMPANY, OF NEW YORK, N. Y., A CORPORATION OF MAINE.

## SHOE-BOTTOM FILLER AND METHOD OF MAKING.

1,114,819.

Specification of Letters Patent.

Patented Oct. 27, 1914.

No Drawing.

Application filed March 7, 1907. Serial No. 361,171.

To all whom it may concern:

Be it known that I, ANDREW THOMA, a citizen of the United States, and resident of Cambridge, in the county of Middlesex and State of Massachusetts, have invented an Improvement in Shoe-Bottom Fillers and Methods of Making, of which the following description is a specification.

My invention is a shoe filler for the bottom cavities of shoes, being one of the varieties or species of shoe bottom filler referred to in my foundation Patent No. 832,002 of September 25, 1906, and capable of manufacture in the form set forth in my application Serial No. 324,368 (now patent No. 945,294, Jan. 4, 1910).

One aim of my present invention is to make it practical from an economic standpoint to use vegetable gums, and another object is to do away with the necessity of dry heat in its use, or at least of such heat as I have preferred to employ in connection with the apparatus disclosed in my Patent No. 808,224. Accordingly, to these ends, I subject a vegetable gum such as is known to the trade as pontianak, or other gums such as almeidina, tuna, chicle, and lower-grade gutta-percha, although these are somewhat more expensive, to a rendering process in a steam-jacketed kettle under the disintegrating influence of free-flowing mineral oil and liquid creosote and resins (the presence of the oils and the fact that a steam-jacketed kettle is used, serving to maintain and insure a low, steady heat), and when the process is wholly completed and the mass is cooled, a very strong, stretchable, rubber-like mass results, having the characteristics of being readily adhesive, tenacious, flexible, waterproof, and cementitious. The disintegration of the gum by the fluxing components mentioned must be entire, and I lay emphasis on this point, as therein resides one of the important discoveries or essentials of my invention. By this means I obtain the qualities of the better class of rubber, and at the same time avoid the necessity of the usual naphtha solution which has been considered necessary for making rubber cement. I obtain a cementitious substance, to be combined with the desired granular body, which is adhesive, cohesive, and elastic, does not require a solvent such as naphtha, is much cheaper than rubber, and much better, as it retains its quality of

cohesion and is therefore a permanently excellent, non-volatile binder for the granular body. The entire and absolute disintegration of the gum by its fluxing components produces an elastic, stretchable sticky mass capable of being mixed with the granular body in the so-called rubber grinding mills, whereby it is compelled to commingle with a large proportion of granular cork for example. The mills act to mix cold the various parts into a uniform mass, the motion or friction of the rolls serving to sufficiently soften the cementitious material or binding agent to facilitate the mixing operation without the use of artificial heat applied either to the binder or to the rolls. This is a great advantage over the preferable process of mixing set forth in my Patent No. 832,002, where the materials have to be maintained hot and fluid. The cold mixing process of my present invention serves to retain in the material the natural strength and tenacity of the binding agent. To take advantage of this feature to the fullest extent, I prefer not to subject the base of vegetable gum to a severe heat, in the rendering process mentioned, but only to a partial heat rendering process, and then to complete the thorough mixing and smoothing of the gum in the mills so as not to destroy the natural strength and tough character of the gums, as would be the case if solely the heat melting method were employed. When these gums are boiled over a high heat, their natural strength and tissue are destroyed and they are rendered very fluid and are practically converted into resins or resinous substances having little or no elasticity. This enables me to secure a filler material of greater tenacity and cohesiveness than would be possible by subjecting the same ingredients to a fluxing and mixing method by heat alone.

I wish it understood that in stating my preferred process or method of manufacture above, I do not limit myself thereto. While it is preferable to employ the heat rendering together with the cold milling, a very satisfactory product may be made solely by the heat rendering process, and likewise solely by the cold milling or smoothing mixing process of the rubber mills.

A great variety of means, such for example as cogum; (i. e. a sticky, coagulated oil) and the long list of recognized equiva-

lents on the market, may be employed to render the gums in question sticky and pasty so that they may be treated by the action of mills and admixed with the granular matter which preferably enters into the composition of shoe filler. In order that my invention may be more definitely apprehended, I will mention a few preferable formulae or relative proportions of the ingredients mentioned. For example, 50 pounds of pontianak, 40 pounds rosin or resinous pitch, 3 gallons of limpid (*i. e.* mobile or free flowing) mineral oil, and three quarters of a gallon of liquid creosote produce good results, slightly more of the mineral oil, say one half gallon additional, being used where the heat treatment alone is resorted to; or 50 pounds pontianak, 30 pounds rosin, and 25 pounds medium *i. e.* very low-melting (*e. g.* gravity from 4 to 5 Twaddell at 180 F.) wax tailings or petroleum residuum. When the milling and mixing is to be done on the mills alone, the rosin and fluxing oil, *i. e.* the mineral oil and creosote in the one case, are first fluxed together by heat before they are added to the gum on the mills, the mixing with the gum taking place on the mills in the same manner as now practised with rubber compounds in regular rubber manufacture.

I have found that the influence of mineral oil in the foregoing compounds is preferable to common vegetable oils, the latter having a peculiar destructive influence upon the gum when fluxed by heat; but whenever the milling process alone is resorted to, vegetable oils, excepting for their higher cost, may be used to advantage in a boiled semi-solid state. So likewise may chemically treated oils of the same sticky, semi-solid nature. Thus good results are secured by mixing 40 pounds of rosin and 2 gallons of mobile or free-flowing mineral oil (which have previously been fluxed together under heat) with 50 pounds of pontianak gum and 8 pounds of thick semi-solid boiled or treated vegetable oil. There are numerous artificial sticky pastes made from oils either by themselves or by their combination with gums or resins, well known in the rubber trade and on the market, which may be added to the vegetable gum in question, within the spirit and scope of my invention.

The compound is milled into a sticky paste and mixed by the milling process with the preponderating amount of granulated cork or the like until it is reduced to the relative stiffness and consistency required for the shoe filler product as set forth in my beforementioned Patent No. 832,002.

One of the advantages resulting from my present invention is that the filler loaf or cake (*i. e.* supposing that the product is put up in that shape as set forth in my before-mentioned patent) can be readily reduced to

the proper consistency for direct application to the shoe bottoms by simply being placed in a steam bath, such for instance as may be provided by an apparatus similar to a glue pot, but having the inner pot shallow and perforated so as to permit the steam and moist vapor to percolate and penetrate through the filler mass, helping quickly to soften and disintegrate the same, and thereby place it in condition to be handled and to be quickly molded into the bottoms of the shoes. The hot moisture, although unable to disturb the binding agent of the mass, helps to soften the same and to separate the material into a workable condition so that it may be handled quickly, not stick to the heated tools, and have a non-resisting, readily moldable and workable character, and nevertheless be quick-setting, permanently tenacious, elastic, and unchangeable in the sense set forth in my first mentioned shoe filler patent.

The method of use is not herein claimed, as the same forms the subject matter of a divisional application, Serial No. 689,395, filed April 8, 1912.

Having described my invention, what I claim as new and desire to secure by Letters Patent is:

1. The method of making a filler compound, consisting of combining a vegetable gum of the character of the so-called rubber-like and pseudo-rubber gums having the general properties herein set forth with a sticky, pasty, fluxing agent through the agency, at least partially, of friction milling under pressure.

2. The method of making the herein described filler compound, consisting of fluxing together mineral oil and resin to make a sticky, pasty fluxing agent, and combining a vegetable gum having the general properties of being rubber-like, and capable of developing a stretchable quality through the agency, at least partially, of friction milling under pressure.

3. The method of making the herein described filler compound, consisting of fluxing together oil and resin, and then combining therewith, by friction milling, at least in part, a gummy base having a rubber-like character until said base is wholly disintegrated and the whole is reduced to a rubber-like mass.

4. The method of making the herein described filler compound, consisting of fluxing together oil and resin, and then combining therewith, by friction milling, at least in part, a gummy base having a rubber-like character until said base is wholly disintegrated and the whole is reduced to a rubber-like mass, and then thoroughly intermixing with said mass a preponderating amount of comminuted filler material.

5. The method of making the herein de-

scribed filler compound, consisting of disintegrating a base containing a resinous vegetable gum, by the agency, at least in part, of heat in the presence of mineral oil, 5 and subjecting the compound to friction milling until thoroughly mixed.

6. The method of making the herein described filler, consisting of fluxing together mineral oil and resin, then combining there- 10 with a rubbery vegetable gum until the latter is wholly disintegrated and reduced to a rubber-like mass, and then introducing granular filler material by friction milling.

7. The method of making the herein described filler compound, consisting of combining a resinous vegetable gum of the kind described and a sticky fluxing agent containing mineral oil by means of moderate heat followed by friction milling until the 20 product is smooth and uniformly pasty.

8. A shoe-bottom filler, consisting of a binder and comminuted filler material mixed together to a semi-solid consistency sluggishly moldable in mass when cold, 25 said binder being derived from a resinous vegetable gum and a fluxing compound containing low-melting petroleum residuum.

9. A shoe-bottom filler, consisting of a binder and comminuted filler material 30 mixed together to a semi-solid consistency sluggishly moldable in mass when cold, said binder being derived from a rubbery mass and a fluxing compound containing low- melting petroleum residuum.

35 10. A filler compound, comprising a melt- able vegetable gum disintegrated in a flux-

ing compound containing mineral oil and creosote.

11. A filler compound, comprising a vegetable gum disintegrated in a fluxing compound containing limpid mineral oil, creosote, and resin. 40

12. A filler compound, comprising a melt- able vegetable gum disintegrated in a flux- 45 ing compound containing wax tailings and resin.

13. A filler compound, comprising pon- tianak and a fluxing agent containing mineral oil and creosote.

14. A filler compound, comprising pon- 50 tianak and a fluxing agent containing resin, mineral oil and creosote.

15. A filler for filling the bottom cavities of shices, comprising a meltable vegetable 55 gum thoroughly admixed to a semi-solid state with filler body material and sticky wax tailings.

16. A shoe bottom filler, comprising a binder of rubber-like vegetable gum com- 60 bined with and wholly disintegrated by an oily fluxing agent, and reduced to a pasty permanently adhesive, tenacious, flexible, waterproof, and cementitious mass, thor- 65oughly mixed with a mass of finely com- minuted filler material.

In testimony whereof, I have signed my name to this specification, in the presence of two subscribing witnesses.

ANDREW THOMA.

Witnesses:

GEO. H. MAXWELL,  
EDWARD MAXWELL.

Copies of this patent may be obtained for five cents each, by addressing the "Commissioner of Patents, Washington, D. C."